# EUROPEAN PATENT SPECIFICATION

(11) **EP 0 853 698 B1**
(45) Date of publication and mention of the grant of the patent: **14.06.2000**
(21) Application number: 96930263.7
(22) Date of filing: 12.09.1996
(51) Int. Cl.: D06M 17/00, D06M 17/04, D06M 17/06, A41D 27/06

(54) **FABRICS COATED WITH ADHESIVE DISSIPABLE BY STEAM**
STOFFE MIT EINER BESCHICHTUNG EINES DURCH DAMPF DISSIPIERBAREN KLEBSTOFFES
TISSUS ENDUITS D'UN ADHESIF DISSIPABLE A LA VAPEUR

(30) Priority: 14.09.1995 GB 9518818
(43) Date of publication of application: 22.07.1998
(73) Proprietor: William Clark & Sons Limited, Maghera, County Londonderry BT46 5RZ (GB)
(72) Inventor: JUDD, Peter, Thomas, St. Albans Herefordshire AL4 9LA (GB); McCORD, Robert, Graffin, Maghera County Londonderry BT46 5RZ (GB)
(74) Representative: McNally, Roisin
(86) International application number: GB9602254
(87) International publication number: WO9710377

(56) References cited:
- BE-A- 699 507
- GB-A- 2 188 566
- US-A- 3 961 125
- US-A- 4 333 980
- PATENT ABSTRACTS OF JAPAN vol. 017, no. 567 (C-1120), 14 October 1993 & JP 05 163603 A (KOOTEC KK), 29 June 1993,

## Description

This invention relates to improvements relating to bonded fabrics, particularly but not exclusively fabrics for use in clothing manufacture.

In the manufacture of clothing such as jackets, several layers of material are brought together to give the jacket a good "shape" and "feel". In places, a jacket can have five layers: outer cloth; interlining, chest canvas, and felt (all known as 'interlinings'); and an innerlining. These layers must be held together to allow the stitching of the layers together and stitching of the fabrics to other parts of the jacket.

Usually, at least some of the layers, especially the outer cloth and one or more of the interlinings, are permanently bonded, or "fused", by an adhesive added thereinbetween. However, fused interlinings can subsequently delaminate unevenly and differential shrinkage can occur upon cleaning, especially after a number of cleaning operations. As such unevenness affects the shape of the outer cloth, such delamination is undesired.

There have been attempts to provide temporarily bonded interlinings, ie. bonded interlinings which are detachable subsequent to the stitching operation. Detachment of the interlining can provide a bespoke look and feel to the clothing, and create a soft handle following the trend towards wearer comfort. Moreover, frequency of cleaning would not be a problem. The initial bonding is still required to provide a fabric which can be immediately and easily sewn together, sewn to other layers and/or sewn to other parts of the jacket.

Documents BE-A-699507, JP-A-5163603, US-A-3961125 and GB-A-2188566 all disclose fabric for use in clothing manufacture wherein two or more layers of fabric are temporarily bonded together by adhesive wherein the adhesive is at least substantially soluble or dissipable by a dry-cleaning solvent or water.

US-A- 3 333 280 and US-A- 4 333 980 disclose the use of small quantities of polyvinylacetate (pva) copolymer as a temporary adhesive for shirt collars and cuffs, removable by dry cleaning and/or laundering the garments in water. However, we have not been able to reproduce these inventions following the teachings in these documents. It is known that pva copolymer is not suitable and does not provide complete delamination of fabric layers for garments which are usually dry cleaned rather than laundered in water, because it is not substantially soluble in the common dry cleaning solvents (such as perchloroethylene). Nor is pva copolymer removed by or dissipated by steaming. The pva copolymer is not therefore completely removed from the garment, and continues to provide some (unwanted) adhesive action or possibly reattachment of the layers. Pressing such fabrics can also lead to unwanted and uneven reattachment of the layers.

An object of the present invention is to obviate or mitigate these disadvantages.

According to an aspect of the present invention, there is provided a fabric having a coating of adhesive thereon adapted to provide temporary bonding of the fabric to one or more other fabrics, wherein the adhesive is wholly or substantially dissipable by steam.

According to the present invention, the adhesive is dissipable by steam. As most clothing garments are steam-pressed at the "pressing off" stage of garment manufacture, the removal of the temporary bonding in this way involves no further steps or equipment in the manufacturing process.

The adhesive or other polymeric material may be a resin/wax mixture; more preferably, a mixture of ethylene vinyl acetate (eva) copolymer resin, and either an eva wax or paraffin wax or a combination thereof. Mixtures of eva copolymer resin and wax can be between 20:80% polymer/wax and 80:20% wax/polymer depending on the melt flow index of the eva polymer selected. The blending of the wax into the resin lowers the viscosity of the resin, allowing the blend to obtain greater flow and to wick into the fabric upon the application of steam.

The quantity of adhesive to be used in the present invention for the coating corresponds substantially to the quantity of adhesive used to provide a permanent bond in prior art multi-layered fabrics. For an interlining fabric for use in the manufacture of jackets, the quantity of adhesive may be 5 to 15 g/m², preferably 5 to 10 g/m². Usually, the minimum amount of adhesive necessary for effect is applied.

The adhesive may be applied to the fabric by any suitable method. Suitable application methods include pastes, dispersions, scattercoat, hot melt and powder point printing or dry powder engraving. Where necessary or desired, the adhesive is coated onto the fabric, but requires 'activation' before being able to bond with other fabrics. Such activation includes heat treatment such as a hot press.

The fabric of the present invention may be used for any suitable purpose including in the manufacture of other fabrics and/or garments. The fabric is particularly suitable for use in clothing manufacture, especially in the manufacture of multi-layered garments such as suits and jackets, where some or all of the interlinings could be similarly coated and bonded. The fabric can be adhered to other parts or layers of the garments before stitching, and then delaminated by steaming. The garments may be cleaned or laundered before sale.

Any number of layers of fabrics of the present invention can be held together as described above.

According to a preferred embodiment of the present invention, the fabric is an interlining, more preferably a haircloth.

According to a second aspect of the present invention, there is provided a method of temporarily bonding two or more layers of fabric together wherein the layers are bonded by applying an adhesive thereinbetween, the adhesive being wholly or substantially dissipable by steam.

Preferably the adhesive is a mixture an eva copolymer resin and either an eva wax or paraffin wax or combination of said waxes.

According to another aspect of the present invention, there is provided a multi-layered clothing garment wherein two or more of the layers of the garment are temporarily bonded by an adhesive as described above. The present invention also extends to a method of manufacture of a multilayered clothing garment as defined in claims 12, 13 and 14 wherein at least two if not all of the layers are temporarily bonded as herein described.

The term "fabric" as used herein includes any woven or non-woven material.

Embodiments of the present invention will now be described by way of example only.

### EXAMPLE

In this example, the adhesive dissipable by steam is a combination or blend of synthetic polymer resin and wax. Ethylene vinyl acetate copolymers having a vinyl acetate content between 8-40% and melt flow index between 0.2 - 3000g/10 mins have been found to be suitable polymer resins. Such resins are compatible with a wide range of waxes, especially eva waxes with a melting range of 70 - 120°C, and paraffin waxes with melting range of 50 - 70°C.

A blend of the above was placed on an interlining base fabric in printed scatter or continuous form. The interlining was placed against an outer fabric and the two heated to a temperature between 60 - 80°C with applied pressure. The heat and pressure caused the blend to flow and fuse to create a bond between the materials. The bond is sufficient to allow the make-up procedure of a garment to continue without detachment of the materials.

The final "pressing-off" stage of the garment production was a steam pressing process. The application of steam and steam pressure with a temperature in excess of 100°C caused the resin/wax blend to rapidly reduce in viscosity and dissipate into the materials. This dissipation or "wicking" action left no blend at the glue line between the materials, destroying the bond created.

## Claims

1. A fabric having a coating of adhesive thereon adapted to provide temporary bonding of the fabric to one or more other fabrics, wherein the adhesive is wholly or substantially dissipable by steam.

2. A fabric as claimed in Claim 1 wherein the adhesive is a resin/wax mixture.

3. A fabric as claimed in Claim 2 wherein the resin/wax mixture is ethylene vinyl acetate copolymer resin and either an ethylene vinyl acetate wax or paraffin wax or a combination thereof.

4. A fabric as claimed in any of the preceding Claims wherein the adhesive requires activation before being able to bond with other fabrics.

5. Use of a fabric as claimed in any of the preceding Claims in clothing manufacture.

6. Use of a fabric as claimed in Claim 5 in the manufacture of suits and jackets.

7. A fabric as claimed in any one of Claims 1 to 4 wherein the fabric is an interlining.

8. A fabric as claimed in Claim 7 wherein the interlining is a haircloth.

9. A method of temporarily bonding two or more layers of fabric together wherein the layers are bonded by applying an adhesive thereinbetween, the adhesive being wholly or substantially dissipable by steam.

10. A multi-layered clothing garment wherein two or more layers of the garment are temporarily bonded by an adhesive as defined in any one of Claims 1 to 4.

11. A multi-layered clothing garment wherein one or more of the layers of the garment is a fabric as claimed in any one of Claims 1 to 4, 7 and 8.

12. A method of manufacturing a multi-layered clothing garment wherein two or more of the garment layers are optionally cut to shape, temporarily bonded together by the adhesive as defined in any of claims 1 to 4, and the layers sewn together, and wherein the garment once finished is then ready to be steam-treated to dissipate the adhesive.

13. A method as defined in claim 12, wherein the finished garment is then steam-treated to dissipate the adhesive.

14. A method of manufacturing a multi-layered garment as defined in Claim 12 or 13 wherein the garment layers are temporarily bonded together by feeding the layers through the hot press.

## Patentansprüche

1. Ein Gewebe mit einer Schicht Klebstoff, der ausgerichtet ist, um das Gewebe vorübergehend mit einem oder mehreren anderen Geweben zu verbinden, wobei der Klebstoff vollständig oder im wesentlichen durch Dampf abbaubar ist.

2. Gewebe gemäß Anspruch 1, wobei der Klebstoff eine Harz-Wachsmischung ist.

3. Gewebe gemäß Anspruch 2, wobei die Harz-Wachsmischung eine Mischung aus Ethylenvinylacetatcopolymerharz und entweder einem Ethylenvinylacetatwachs oder einem Paraffinwachs oder einer Kombination davon ist.

4. Gewebe gemäß einem der vorhergehenden Ansprüche, wobei der Klebstoff aktiviert werden muß, bevor er sich mit anderen Geweben verbinden kann.

5. Verwendung eines Gewebes gemäß einem der vorhergehenden Ansprüche in der Kleidungsherstellung.

6. Verwendung eines Gewebes gemäß Anspruch 5 bei der Herstellung von Anzügen und Jacken.

7. Gewebe gemäß einem der Ansprüche 1 bis 4, wobei das Gewebe ein Futterstoff ist.

8. Gewebe gemäß Anspruch 7, wobei der Futterstoff ein Haartuch ist.

9. Ein Verfahren zum vorübergehenden Verbinden von zwei oder mehr Schichten von Gewebe, wobei die Schichten verbunden werden, indem ein Klebstoff dazwischen aufgetragen wird, wobei der Klebstoff vollständig oder im wesentlichen durch Dampf abbaubar ist.

10. Ein mehrschichtiges Kleidungsstück, wobei zwei oder mehr Schichten des Kleidungsstücks vorübergehend durch einen wie in einem der Ansprüche 1 bis 4 festgelegten Klebstoff verbunden werden.

11. Ein mehrschichtiges Kleidungsstück, wobei eine oder mehr Schichten des Kleidungsstücks aus einem in einem der Ansprüche 1 bis 4, 7 und 8 festgelegten Gewebe bestehen.

12. Verfahren zur Herstellung eines mehrschichtigen Kleidungsstücks, wobei zwei oder mehr Schichten je nach Bedarf zugeschnitten, vorübergehend mittels des Klebstoffes gemäß einem der Ansprüche 1 bis 4 verbunden und die Schichten zusammengenäht werden, und wobei das fertiggestellte Kleidungsstück dann mit Dampf behandelt werden kann, um den Klebstoff abzubauen.

13. Verfahren gemäß Anspruch 12, wobei das fertiggestellte Kleidungsstück dann mit Dampf behandelt wird, um den Klebstoff abzubauen.

14. Verfahren zur Herstellung eines mehrschichtigen Kleidungsstücks gemäß Anspruch 12 oder 13, wobei die Schichten des Kleidungsstücks vorübergehend verbunden werden, indem die Schichten der Heißpresse zugeführt werden.

## Revendications

1. Un tissu recouvert d'un enduit d'adhésif prévu pour procurer le collage temporaire du tissu à un autre tissu au moins, dans lequel l'adhésif peut être entièrement ou sensiblement dissipé grâce à de la vapeur.

2. Un tissu selon la revendication 1 dans lequel l'adhésif est un mélange résine/cire.

3. Un tissu selon la revendication 2 dans lequel le mélange résine/cire est de la résine copolymère éthylène/acétate de vinyle et soit une cire éthylène/acétate de vinyle soit de la cire de paraffine soit une combinaison de celles-ci.

4. Un tissu selon n'importe lesquelles des revendications précédentes dans lequel l'adhésif nécessite d'être activé avant de pouvoir coller à d'autres tissus.

5. Utilisation d'un tissu selon n'importe lesquelles des revendications précédentes dans la fabrication d'habillement.

6. Utilisation d'un tissu selon la revendication 5 dans la fabrication de costumes et de vestes.

7. Un tissu selon une quelconque des revendications 1 à 4 dans lequel le tissu est un entoilage.

8. Un tissu selon la revendication 7 dans lequel l'entoilage est un tissu à poil.

9. Un procédé pour coller temporairement ensemble deux couches au moins de tissu dans lequel les couches sont collées en appliquant un adhésif entre celles-ci, l'adhésif pouvant être entièrement ou sensiblement dissipé grâce à de la vapeur.

10. Un vêtement d'habillement multicouche dans lequel deux couches au moins du vêtement sont collées temporairement par un adhésif comme le définit une quelconque des revendications 1 à 4.

11. Un vêtement d'habillement multicouche dans lequel une des couches du vêtement au moins est un tissu selon une quelconque des revendications 1 à 4, 7 et 8.

12. Un procédé de fabrication d'un vêtement d'habillement multicouche dans lequel deux des couches de vêtement au moins sont coupées en forme de façon optionnelle, collées temporairement ensemble par l'adhésif comme le définissent n'importe lesquelles des revendications 1 à 4, et les couches cousues ensemble, et dans lequel le vêtement une fois fini est ensuite prêt à être traité à la vapeur pour dissiper l'adhésif.

13. Un procédé comme le définit la revendication 12, dans lequel le vêtement fini est ensuite traité à la vapeur pour dissiper l'adhésif.

14. Un procédé de fabrication d'un vêtement multicouche comme le définit la revendication 12 ou 13 dans lequel les couches de vêtement sont collées temporairement ensemble en faisant passer les couches au travers de la presse à chaud.
